

## 1

3,447,942

### PREPARATION OF SENSITISED PHOTOGRAPHIC PAPER

Albert Edward Harris and Frank R. Tolhurst, Ilford, Essex, England, assignors to Ilford Limited, Ilford, Essex, England, a British company

No Drawing. Filed Dec. 1, 1965, Ser. No. 510,967  
Claims priority, application Great Britain, Dec. 23, 1964,  
52,236/64

Int. Cl. G03c 1/88; B32b 29/06  
U.S. Cl. 117—4

4 Claims

#### ABSTRACT OF THE DISCLOSURE

Sensitised photographic paper having reduced tendency to curl when cut into discrete sheets is prepared by coating one face of a paper web with an aqueous gelatino-silver-halide emulsion, drying the emulsion coating, and then contacting the other non-coated face of the web with the heated surface of a drum or drums for not less than 15 seconds, the temperature of the drum or drums being between 100 and 200° F. and then cutting the coated web into discrete sheets.

This invention relates to the preparation of sensitised photographic paper carrying a gelatino silver halide emulsion and in particular to a method of producing such paper with improved curl characteristics.

Sensitised photographic paper is made by coating a gelatino-silver-halide emulsion on to a strong paper base web. A web of photographic paper after it has been coated with the gelatino-silver-halide emulsion and dried, is normally cut up in to discrete sheets and stored in boxes. Unless very stringent precautions are taken regarding the relative humidity of the atmosphere in which the sheets are to be stored, it is found that when the sheets are removed from the boxes they will exhibit face curl, that is to say the paper will be curled towards the emulsion-coated side. This type of curl is called preprocessing curl and is to be distinguished from the curl usually produced after sheet material has been processed.

It is an object of the present invention to provide a method of producing sensitised photographic paper which reduces or eliminates such preprocessing curl.

According to the present invention there is provided a method of producing sensitive photographic paper which comprises coating one face of a paper web with an aqueous gelatino-silver-halide emulsion, drying the gelatino-silver-halide emulsion coating, and thereafter contacting the other face of the web with at least one smooth surfaced heated drum, the temperature of the drum or drums being between 100° F. (37° C.) and 200° F. (93° C.) and the total contact time between any portion of the web and the heated drum or drums being not less than 15 seconds, and thereafter cutting the web to discrete sheet form.

The preferred method for carrying out this invention comprises coating one face of a paper web with an aqueous gelatino-silver-halide emulsion, drying the gelatino-silver-halide coating, and then, continuously with the coating, guiding the coated paper web on to one or more

## 2

smooth metal-surfaced heated drums rotating at a peripheral speed substantially equal to the rate of travel of the webs, so that the other face of the coated paper web contacts the peripheral surface of the said heated drum or drums and is carried around a portion of the circumference of the heated drum or drums in close contact therewith, the temperature of the heated drum or drums being between 100° F. (37° C.) and 200° F. (93° C.) and the total contact time between any portion of the web and the heated drum or drums being not less than 15 seconds and thereafter cutting the web to discrete sheet form.

The contact time during which any portion of the web should, for optimum results, be in contact with the heated drum or drums depends on the temperature. For example, if the temperature of the drum or drums is 130° F. a total contact time of about 100 seconds is generally found desirable but if the temperature of the drum or drums is 170° F. only 20 seconds total contact time may be necessary.

It has been found possible to store sensitised photographic paper, prepared according to this invention, in sheet form in boxes for several months in an atmosphere having a relative humidity of 40% without the sheet material showing any important preprocessing curl when it is removed from the box.

In order to determine if the heating of freshly coated photographic paper to comparatively high temperatures had any deleterious effects on the sensitometric properties of the emulsion freshly coated Ilford Chlorobromide Paper No. 2 (the word Ilford is a registered trademark) was heated to 200° F. for various lengths of time. The table below shows that the sensitometric properties of the emulsion are not adversely affected.

TABLE

| Oven temperature<br>(° F.) | Time<br>(sec.) | Speed 0.7<br>above fog level | Contrast | D <sub>max</sub> |
|----------------------------|----------------|------------------------------|----------|------------------|
| 40                         | 0              | 2.37                         | 1.75     | 1.94             |
| 200                        | 10             | 2.41                         | 1.65     | 1.89             |
| 200                        | 30             | 2.39                         | 1.65     | 1.92             |
| 200                        | 60             | 2.39                         | 1.75     | 1.97             |

We claim as our invention:

1. A method of producing sensitive photographic paper which comprises coating one face of a paper web with an aqueous gelatino-silver-halide emulsion, drying the gelatino-silver-halide emulsion coating, and thereafter contacting the other face of the web with at least one smooth surfaced heated drum, the temperature of the drum or drums being between 100° F. (37° C.) and 200° F. (93° C.) and the total contact time between any portion of the web and the heated drum or drums being not less than 15 seconds, and thereafter cutting the web to discrete sheet form.

2. A method according to claim 1 wherein the drum or drums are metal surfaced.

3. A method according to claim 1 wherein the drum or drums are revolving during the time the paper is in contact with them.

4. A method of producing sensitive photographic paper which comprises coating one face of a paper web

with an aqueous gelatino-silver-halide emulsion, drying the gelatino-silver-halide coating, and then, continuously with the coating guiding the coated paper web on to one or more smooth metal-surfaced heated drums rotating at a peripheral speed substantially equal to the rate of travel of the webs, so that the other face of the coated paper web contacts the peripheral surface of the said heated drum or drums and is carried around a portion of the circumference of the heated drum or drums in close contact therewith, the temperature of the heated drum or drums being between 100° F. (37° C.) and 200° F. (93° C.) and the total contact time between any portion of the web and the heated drum or drums being not less than 15 seconds and, thereafter cutting the web to discrete sheet form.

## References Cited

## UNITED STATES PATENTS

|   |           |         |                    |        |        |
|---|-----------|---------|--------------------|--------|--------|
| 5 | 2,620,285 | 12/1952 | Rose               | -----  | 117—34 |
|   | 2,659,680 | 11/1953 | Gray               | -----  | 117—34 |
|   | 2,865,792 | 12/1958 | Gray               | -----  | 117—34 |
|   | 2,269,169 | 1/1942  | Van Derhoef et al. | 117—34 |        |
|   | 3,227,578 | 1/1966  | Parkin             | -----  | 117—34 |

MURRAY KATZ, Primary Examiner.

10

U.S. Cl. X.R.

96—85; 117—34, 66, 156